

E. A. ASHCROFT,

APPARATUS FOR THE ELECTROLYTIC MANUFACTURE OF LIGHT METALS AND REACTION  
PRODUCTS THEREOF.

APPLICATION FILED MAR. 12, 1912.

1,204,234.

Patented Nov. 7, 1916.

3 SHEETS—SHEET 1.



Fig. 1.

WITNESSES

Walter Albre

W. E. Keib

INVENTOR

Edgar Arthur Ashcroft  
BY

Horowitz and Horowitz  
his ATTORNEYS

E. A. ASHCROFT.

APPARATUS FOR THE ELECTROLYTIC MANUFACTURE OF LIGHT METALS AND REACTION  
PRODUCTS THEREOF.

APPLICATION FILED MAR. 12, 1912.

1,204,234.

Patented Nov. 7, 1916.

3 SHEETS—SHEET 2.



WITNESSES

Walter A. Astor  
W. E. Kins

INVENTOR

Edgar Arthur Ashcroft  
BY

Strawn and Strawn  
his ATTORNEYS

E. A. ASHCROFT.

APPARATUS FOR THE ELECTROLYTIC MANUFACTURE OF LIGHT METALS AND REACTION  
PRODUCTS THEREOF.

APPLICATION FILED MAR. 12, 1912.

1,204,234.

Patented Nov. 7, 1916.

3 SHEETS—SHEET 3.

Fig. 3.



WITNESSES

Walter Abbr.  
M. E. Neir

INVENTOR

Edgar Arthur Ashcroft  
*BY*

Horace and Horace  
his ATTORNEYS

# UNITED STATES PATENT OFFICE.

EDGAR ARTHUR ASHCROFT, OF LONDON, ENGLAND.

## APPARATUS FOR THE ELECTROLYTIC MANUFACTURE OF LIGHT METALS AND REACTION PRODUCTS THEREOF.

1,204,234.

Specification of Letters Patent. Patented Nov. 7, 1916.

Application filed March 12, 1912. Serial No. 683,377.

*To all whom it may concern:*

Be it known that I, EDGAR ARTHUR ASHCROFT, a subject of the King of Great Britain and Ireland, and residing at 99 5 Buckingham Palace road, in the county of London, England, and of Sande Gaard, Balestrand, Sogn, Norway, electrochemical engineer, have invented new and useful Improvements in and Apparatus for the Electrolytic Manufacture of Light Metals and 10 Reaction Products Thereof, of which the following is a specification.

The object of my invention is to effect the manufacture of the class of metals known as 15 light metals, and particularly sodium and potassium, or reaction products thereof (or both) in a very efficient and economical manner.

My invention relates more particularly to 20 processes in which a salt of an alkali metal (or a mixture of such salts) is electrolyzed in a first cell over a cathode of liquid metal, the resulting alloy of the alkali metal and liquid metal constituting an anode in a second cell 25 in which an electrolyte in accordance with the required product is employed, but it is not confined to such processes and may be utilized for any electrolytic production of light metals from fused metals and it is 30 especially adapted for use in effecting the economical electrolysis of fused amids of the alkali metals with, or without, excess metals dissolved therein as described in my applications Ser. Nos. 683,376, 683,379.

Great difficulties have been experienced 35 in practice in recovering, by electrolysis alkali metals from fused metals of all kinds and more particularly is this the case when an anode of soluble alloy is used. For instance if more than an extremely small 40 cathode surface (or any surface in electrical contact with the cathode) be exposed in the melt no metal at all will appear while if too great a distance between cathode and 45 anode, or too high current density at any part of the anode, exist, effects equally fatal to success will arise.

In carrying out my invention I have 50 found by research that it is impossible to obtain the necessary conditions in practice without special devices in the second cell which I now describe under two alternative methods either of which is effective. According to the first of these methods, in 55 order to obtain the aforesaid conditions as

regards current density and resistance, the arrangement may be such that the required product collects upon a number of small electrode parts, or points, arranged symmetrically over a given anode area, and in 60 order to collect the product and remove it rapidly from the field of further action, a constant flow of electrolyte in a very shallow layer over the anode is carried from a reservoir, preferably by means of a rotating worm pump, past the said small parts, or points. By this means it is practicable to remove the product of electrolysis and carry it at once out of the field of further reaction over a weir, or overflow, to a receptacle, or 70 chamber, in which the product collects and from which it can be withdrawn by a suitably placed overflow pipe, or be otherwise removed, for example by ladles. The electrolyte reservoir may be separate from the 75 main casting, or form part thereof. It is convenient to so direct the discharge from the pump into the cell that rotary motion of the electrolyte is set up and maintained. The product being a light metal 80 (for instance sodium) it floats on the electrolyte and remains in the upper part of the collecting chamber being there conveniently aggregated into a floating mass, while the associated electrolyte, being heavier, 85 falls to the bottom of the said receptacle, or chamber, and by means of passages, passes back to the reservoir, thus maintaining a continuous flow and circulation of the electrolyte past the cathode and over the anode 90 surface and agglomerating the produced metal in a place where it is not subjected to secondary reactions, but which is convenient for its economical collection. The aforesaid collecting chamber is preferably maintained 95 at a lower temperature and may, if desired, be artificially cooled as by a coil of pipe 17 through which a cooling medium may be circulated. This prevents re-solution of the metal and will throw out of solution again 100 some of the metal which may have been dissolved in the electrolyte. The produced alkali metals may be removed continuously, or intermittently, from such outlet in any 105 desired manner but preferably are allowed to run off continuously into a small receptacle. The said arrangement also facilitates the automatic separation of any small quantities of impurities (such as lead) which may be deposited with the alkali metal by 110

reason of the gravitation of the lead through the floating body of fused alkali metal, which I have specifically observed.

The hereinbefore described arrangement is equally useful when reaction products such as amids and the like are produced *in situ* in the second cell by electrolysis as described in the specification of my co-pending application Ser. No. 555530 and under 10 my application Ser. No. 683,376, for it is found that without such proportions and disposition of the parts only very inefficient electrolysis takes place. Extensive experiments which I have made have established 15 the practical advantages of this arrangement over any other. The cathode is preferably constituted by small rods (preferably of nickel) of about 10 millimeters diameter brought to a conical and rounded end (an 20 inverted parabola), or flat, and carried by a plate (preferably of copper) provided with means by which the position of the cathode can be adjusted to regulate its distance from the anode and the extent of surface in contact with the electrolyte. The overflow is 25 preferably arranged at the center of the cell, and the small rods of the cathode are preferably arranged in circumferential rows. The metal which collects at the top of the 30 receptacle into which the overflow takes place can be drawn off by a pipe projecting into the upper part of the said receptacle, or by other suitable means, such for instance as ladles. If the produced, or dissolved, 35 metal be reacted *in situ* the derived product, instead of the metal, is drawn off by the overflow pipe. Such derived products may, for example, be amid, cyanamid, cyanid, or hydrate.

40 Other forms of cell embodying the same leading principles may be employed for carrying out my invention, for instance I may use a rectangular cell with the weir, or overflow, and receptacle at one end and the electrolyte inlet at the other end, the cathode parts being disposed in rows to suitably equalize the distribution of the current over the anode surface. The electrolyte reservoir, when a derivative of the alkali metal 45 is required, is provided with means for introducing the necessary reagent, or reagents, (for instance ammonia, or ammonia and carbon, benzol, or other hydrocarbon, or dicyan-diamid, trimethyl-amin, hydrocyanic acid, or the like) and with an outlet from 50 which the derivatives can be drawn off from the reservoir, or from the receptacle, as required. An outlet is provided from which the produced gases pass off, these being conducted preferably first to the interior of the 55 second cell and finally to an outlet in the center of that cell so that the gaseous products (for instance hydrogen, or hydrogen and ammonia gas,) will maintain an atmosphere of such gas, or gases, in the said cell

and may, in certain gases, promote further reactions. The second cell is of course provided with inlet and outlet passages for the circulating alloy constituting the anode.

When alloys of alkali, or other light, 70 metals are used for this process, they may be produced by any known, or suitable, means but I prefer the means described under my application Ser. No. 683,375. When alkali amid, or other compound, is electrolyzed an insoluble anode of nickel, or steel, 75 may be used and special precautions as to temperature and other conditions are taken as described under my application Ser. No. 683,379.

80 Figures 1 and 2 of the accompanying drawings represent in longitudinal vertical section and plan, respectively, a second cell in position together with a first cell and common alloy base and reservoir for continuous production of the desired product, the said first cell being of the type described under my application Ser. No. 683,375. Fig. 85 3 is a vertical section of a modified form of the secondary cells in which modification the reservoir is arranged separately of the secondary cell, but suitably connected thereto.

90 1 represents the first cell and 2, the second cell containing the alloy 3, and the electrolyte 4, in a thin layer, thereon.

95 5 are the cathode rods.

6 is the alloy pump.

7 is the reservoir for electrolyte which reservoir constitutes also the pump chamber, and is shown as being within the cell 2, 100 and 8 are the circulating passages and collecting chamber constituting also a part of the reservoir of electrolyte.

9 is the weir over which the electrolyte flows.

10 is the pump for circulating the electrolyte which is discharged against the curved plate 15, so that rotary motion of the electrolyte is set up and maintained in the cell.

110 11 is the overflow for alkali metal, and 12 is the small kettle for receiving the alkali metal.

16 is a pipe by means of which the necessary reagent or reagents can be admitted to 115 the cell 2.

120 In the arrangement shown in Fig. 3, the same parts are employed but the alloy reservoir 7, is exterior to the cell 2, and of larger dimensions. It is connected to the pump 10, and to the collecting chamber below the weir 9, by means of pipes 8 and 13, and a gas pipe 14, connects the free space in the reservoir to that in the cell 2, and permits the free passage of hydrogen, ammonia, or the like.

125 In the second of the aforesaid methods which I may employ for effecting the same objects the electrolyte is contained to a considerable depth in the second cell above the melted alloy and the circulating reservoir is

dispensed with. The necessary restriction of the cathode area immersed in the electrolyte and the convenient collection of the produced metal, or other product, are obtained in any suitable way.

The aforesaid restriction of the area of the immersed cathode is necessary for successful working in such a process and the mechanical and electrical constants of the known 10 metals which can be employed for the cathode (for example, copper, nickel, and the like) are such that the desired result can only be obtained by one, or other, of the hereinbefore described means.

15 In the first described means the circulating reservoir 7, may be either inside the cell 2, as illustrated in Fig. 1, (which arrangement is convenient when producing metals with a high melting electrolyte such as cyanid or the like) or exterior to the cell, as 20 illustrated in Fig. 3, which is convenient when using a low melting electrolyte such as amid or caustic alkali.

In the second described means the introduced gas may be either an inert gas such as 25 hydrogen (for example when metallic products are required), or an active gas such as ammonia, or nitrogenous, or carbonaceous, gas such as benzol, trimethylamin, HCN, or 30 steam, or the like, or any, or all, of such agents, which will react with the produced nascent metal producing the desired derivative cyanid, cyanamid, amid, or hydrate.

It will be understood that my invention 35 can be employed for the obtainment of alkali metals, or derivatives thereof, (or both such metals and derivatives) from alloys of such metals, with other metals (for instance with lead) however such alloys may have 40 been obtained, or it can be employed for the electrolytic production of alkali metals from electrolytes such as amids, cyanids, and the like, using suitably disposed insoluble anodes.

45 It will also be understood that the hereinbefore described process may be usefully combined in various ways with the processes

described under my applications Ser. Nos. 683,375; 683,376; 683,378 and 683,379, according to the final products required and 50 economical conditions generally.

In the following claims the expression "alkali metal products" includes alkali metals themselves as well as reaction products therefrom.

55 What I claim is—

1. An electrolytic apparatus of the character described having only an extremely small cathode area exposed in the electrolyte and in close proximity to the anode, and 60 means for circulating the electrolyte in a thin layer over the surface of the anode.

2. An electrolytic apparatus of the character described having only an extremely small cathode area exposed in the electrolyte 65 and in close proximity to the anode, an overflow chamber for the electrolyte and a pump for returning the latter to the electrolytic cell.

3. An electrolytic apparatus of the character described having only an extremely small cathode area exposed in the electrolyte and in close proximity to the anode, a collecting chamber inside the cell for the electrolytic product and means for gathering 75 the latter in said collecting chamber, together with means for cooling the liquids therein, for the purpose specified.

4. An electrolytic apparatus of the character described having only an extremely 80 small cathode area exposed in the electrolyte and in close proximity to the anode, an overflow chamber for the electrolyte arranged to maintain the latter in a thin layer over the surface of the anode, and means for circulating the electrolyte from the overflow chamber to the electrolytic cell.

In testimony whereof I have signed my name to this specification in the presence of two subscribing witnesses.

EDGAR ARTHUR ASHCROFT.

Witnesses:

ULYSSES J. BYWATER,

PAUL ARRAS.